

## UNITED STATES PATENT OFFICE.

ALBERT WITTIG, OF BERLIN, GERMANY.

## METHOD OF MANUFACTURING ALLOYS FROM IRON.

No Drawing.

Application filed May 7, 1924. Serial No. 711,744.

*To all whom it may concern:*

Be it known that I, ALBERT WITTIG, a citizen of Germany, and a resident of Berlin, Germany, have invented Improvements in a 5 Method of Manufacturing Alloys from Iron, of which the following is a specification.

My invention relates to an improved method of manufacturing certain iron alloys free from phosphorus and arsenic.

10 The commercial iron alloys hitherto employed in the iron metallurgy for refining purposes, such as ferromolybdenum, ferro-vanadium, ferro-wolfranium, ferro-chromium and the like frequently contain a certain 15 percentage of phosphorus and arsenic, which are objectionable and sometimes even render the alloys useless as regards the purpose they are mainly intended for. These impurities originate from the raw ores or materials employed for producing the elementary metals such as molybdenum, wolfram and the like therefrom and on account of difficulties hitherto unavoidable in the process of producing the said metals such impurities remain 20 in the latter and, therefore, are also present in the iron alloys to be made by melting together iron and the said refining metals.

25 The object of my invention is to produce alloys of the kind, which are free from impurities such as phosphorous and arsenic, and to thereby improve the quality of such alloys and the commercial and technical value thereof.

30 The underlying chemical principle of my invention or method is this:—that both phosphorus compounds and arsenic compounds can be detected in acid solutions by means of zirconium salts and that upon 35 addition of a zirconium salt or compound to such a solution both phosphorus and arsenic are precipitated therein in the form of an insoluble zirconium compound or salt.

40 In accordance therewith I treat a suitable 45 solution of the refining metals, such as wolfram, molydenum, vanadium, uranium, chromium, copper and the like with soluble zirconium compounds or salts in order to precipitate and subsequently separate there-

from phosphorus and arsenic and then I employ the thus purified solution for the production of the refining metal or metals contained in said solution in the usual manner and for the purpose of making ferro-alloys therefrom.

45 The chemical nature of the zirconium salts or compounds I employ according to my invention for the precipitation purpose is entirely immaterial. Generally speaking zirconium salts of the mineral acids may be used, but just as well hydroxides, carbonates or basic sulphates of zirconium may be employed instead. I gradually add the zirconium compound to the acid solution of the refining metal after having ascertained the 50 existence or the percentage of phosphorus and arsenic therein, in order to precipitate the latter.

55 The subsequent operations are to be carried out in the customary manner and need no description in order to not unnecessarily burden this specification.

60 In cases where impurities of the natural zirconium minerals such as iron, silicic acid, titanium and the like, do not have any prejudicial effect, also such impure minerals having been properly broken up or rendered soluble before, may be employed or even any suitable intermediate products thereof may be utilized for the purpose of my invention.

65 It will be evident that my invention, whilst still being adhered to in its main essentials, may be varied and adapted in many ways, according to the several requirements desired, or most suitable under different circumstances.

70 What I claim is:—

75 The method of purifying a solution of an iron alloying metal, such as vanadium, chromium, titanium, molybdenum and the like by adding thereto a suitable zirconium compound or salt for the purpose of precipitating any phosphorus and arsenic present in such solution, substantially as set forth.

80 In testimony whereof I have signed my name to this specification.

ALBERT WITTIG.